

# United States Patent [19]

Horvath, Jr. et al.

[11] 3,997,370  
[45] Dec. 14, 1976

[54] **METHOD OF HOT REDUCING FERROUS AND FERROUS ALLOY PRODUCTS WITH COMPOSITE MARTENSITIC NODULAR CAST CHILL IRON ROLLS**

[75] Inventors: **Paul J. Horvath, Jr.**, Whitehall; **John A. Gibbon**, Center Valley, both of Pa.

[73] Assignee: **Bethlehem Steel Corporation**, Bethlehem, Pa.

[22] Filed: **Nov. 17, 1975**

[21] Appl. No.: **632,872**

[52] U.S. Cl. .... **148/12 R**; 29/132; 29/196.1; 148/34

[51] Int. Cl.<sup>2</sup> .... **C22F**

[58] Field of Search .... 148/34, 12.4, 12.1, 148/12.3, 12 D, 12 F, 12 EA, 12 E, 12 A; 29/196.1, 148.4, 132

## [56] References Cited

### UNITED STATES PATENTS

|           |         |                   |       |        |
|-----------|---------|-------------------|-------|--------|
| 2,129,683 | 9/1938  | Gontermann et al. | ..... | 148/34 |
| 3,623,850 | 11/1971 | Horvath, Jr.      | ..... | 148/34 |
| 3,670,381 | 6/1972  | Schoffmann        | ..... | 29/132 |
| 3,855,015 | 12/1974 | Nemoto et al.     | ..... | 148/34 |
| 3,894,325 | 7/1975  | Maruta et al.     | ..... | 148/34 |

Primary Examiner—W. Stallard  
Attorney, Agent, or Firm—Joseph J. O'Keefe; William B. Noll

## [57] ABSTRACT

This invention is directed to a method of hot reducing ferrous and ferrous alloy products, such as plates, strip, bars and rods, where such products are heated to temperatures in excess of 1900° F and subsequently reduced at temperatures within the range of about 900° and the initial heating temperature. More particularly, this invention relates to the method of effecting said hot reducing at such temperatures by means of composite, martensitic, nodular graphite chill cast iron rolls. Such rolls are characterized by (1) an average surface hardness of at least about 76 Shore-C, (2) a thermal-crack-resistant chill cast surface portion consisting essentially of, by weight, about 3.00% to 3.70% carbon, about 0.35% to 1.25% manganese, about 1.0% to 2.0% silicon, about 3.75% to 5.75% nickel, about 0.75% to 1.35% chromium, about 0.40 to 1.10% molybdenum, about 0.3% to 0.08% magnesium, balance iron and incidental impurities, and (3) a core portion comprising a ferrous alloy.

5 Claims, No Drawings

**METHOD OF HOT REDUCING FERROUS AND FERROUS ALLOY PRODUCTS WITH COMPOSITE MARTENSITIC NODULAR CAST CHILL IRON ROLLS**

**BACKGROUND OF THE INVENTION**

This invention is directed to an improved composite chill cast iron roll of the type disclosed in U.S. Pat. No. 3,623,850, issued Nov. 30, 1971 to Paul J. Horvath, Jr. More particularly this invention relates to a new use of such rolls in the hot reduction of ferrous and ferrous alloy products, such as plates, strip, bars and rods. These rolls, as a result of the combination of chemistry, manufacturing sequence, and post treatment, may be characterized as composite martensitic, nodular graphite, chill-cast iron rolls.

Since the original development by Horvath, such rolls have gained much notoriety for their performance in cold mills, or in cold rolling applications. Their outstanding performance has been attributed to the ability of such rolls to resist marking, bruising and spalling, while being readily redressed for further service. However, with cold rolling applications, heat, hence thermal fatigue and cracking, is not a problem.

Rolling mill design has developed over the years into a complex science having many facets to it. For example, cold rolling applications, such as reviewed in U.S. Pat. No. 3,623,850, and hot rolling applications are just two of such facets. Different criteria must be used to determine roll design, such as material selection, properties and capabilities of the roll. In other words, a roll was designed for a specific rolling application because it possessed the properties needed for such application. As indicated above, resistance to thermal fatigue or cracking is a major consideration in determining suitability of a roll for use in hot rolling applications. As a consequence, roll manufacturers, when designing rolls for hot mill applications, particularly for the first several stands of a hot strip mill where the strip temperatures exceed about 1800° F, maintained the shell hardness below a specified value.

In the publication, *Roll Specifications For Finishing Stands of a Modern Continuous Hot Strip Mill*, by John M. Dugan, published by the Association of Iron and Steel Engineers, copyright 1970, the author indicates that the shell hardness of the rolls in the initial stand vs. final stand of a hot mill finishing train will vary by about 7 points on the shore "C" hardness scale. That is, where the temperature of the strip is hottest, the lower hardness roll, i.e. about 75 shore C, is used.

While the shell hardness of a work roll is a prime consideration in the selection of a roll, there are others. For instance, the article entitled, "Cause and Prevention of Hot Strip Work Roll Banding," by Charles E. Peterson and published in the Iron and Steel Engineer Year Book, 1956, offers three possible solutions to the banding problem in a hot mill. Banding, as defined by the author "occurs primarily on the rolls of the first two finishing stands, [and] is caused by the adhesion of sizeable patches of scale on the roll surface. Generally the scale patches are elongated in the direction of rolling, giving the appearance of bands." His solution is (1) effective scale removal from the strip, (2) selection of roll material combining high hardness with freedom from graphite, and (3) adequate coolant to keep rolls as cold as possible.

Faced with these prejudices, the prior art settled for cast steel rolls, a graphite free roll having a nominal composition of 1.7C—1.0Cr—1.7Ni-Fe. However, such rolls are limited in the quantity of product that can be rolled, and by the frequent dressing required to prepare the roll once again for service. To improve the usable work life of their rolls, roll makers began to look to high chromium rolls. Typically these rolls contain about 12 to 20% chromium and are characterized by a Shore-C hardness of between about 60 and 75. While the usable life of a hot mill roll had been increased with the introduction of the high-chromium roll, the premium cost of the highly alloyed chromium rolls made their selection a costly alternative. Moreover, the high chromium roll is sensitive to thermal conditions in the mill and thereby frequently requiring cutdowns because of excessive fire cracking.

Confronted by these facts, including the high cost of an alternative answer, a different approach was needed. It was discovered that a cast iron roll, having a shell portion containing nodular graphite in a martensitic matrix, with an average surface hardness of at least 76 Shore-C, could be used effectively in the hot reduction of ferrous and ferrous alloy products, such as strip, plates, bars and sheet. This was particularly dramatic where the temperatures of the workpiece exceeded about 1800° F. Finally, the cost of such rolls was comparable to that of the presently used cast steel or cast iron rolls, and considerably below the cost of the chromium rolls.

**BRIEF SUMMARY OF THE INVENTION**

This invention is directed to a new use for a composite martensitic, nodular graphite, chill-cast iron roll, more particularly to the method of using such roll for the hot reduction of ferrous and ferrous alloy products, such as plates, strip, bars and rods. In hot rolling applications where the work rolls come in contact with a workpiece which has been heated prior to reduction to temperatures in excess of 2200° F, thermal shock, resulting in cracking, can occur.

The present invention is the result of the discovery that a composite martensitic, nodular graphite, chill-cast iron roll is resistant to thermal cracking while possessing the further attributes necessary for a work roll in a hot rolling application. The roll of this invention is characterized by a surface portion having a hardness of at least 76 Shore-C and consisting essentially of, by weight, about 3.00 to 3.70% carbon, about 0.35 to 1.25% manganese, about 1.0 to 2.0% silicon, about 3.75 to 5.75% nickel, about 0.75 to 1.35% chromium, about 0.40 to 1.10% molybdenum, about 0.03 to 0.08% magnesium, the balance iron and incidental impurities, and a core portion comprising a ferrous alloy whose chemistry and mechanical properties are metallurgically compatible with the chemistry and properties of said surface portion.

**DESCRIPTION OF PREFERRED EMBODIMENT**

The work roll of this invention, for which a new use has been found in hot rolling applications, may be characterized as a composite martensitic, nodular graphite, chill-cast iron roll. Such roll is comprised of a thermal-crack-resistant annular chill surface portion consisting essentially of, by weight, about 3.00% to 3.70% carbon, about 0.35% to 1.25% manganese, about 1.0% to 2.0% silicon, about 3.75% to 5.75% nickel, about 0.75% to 1.35% chromium, about 0.40% to 1.10% molybdenum,

about 0.03% to 0.08% magnesium, balance iron and incidental impurities, whose surface has a hardness of at least 76 Shore-C, and a core portion comprising a cast iron or ferrous alloy.

Within such broad composition range there is a preferred chemistry to give optimum properties, namely,

|            |                |   |
|------------|----------------|---|
| Carbon     | 3.10% to 3.40% | 5 |
| Manganese  | 0.45% to 0.75% |   |
| Silicon    | 1.35% to 1.65% |   |
| Nickel     | 3.90% to 4.30% |   |
| Chromium   | 0.90% to 1.30% |   |
| Molybdenum | 0.55% to 0.80% |   |
| Magnesium  | 0.03% to 0.08% |   |
| Iron       | balance.       |   |

It will be appreciated that within the broad and preferred chemistry ranges a proper relationship must be established among the several elements. For instance, several of the elements are critical in the formation and depth of the chill portion containing nodular graphite. Carbon must be present in an amount over and above that which will form as carbides. Thus, if such carbide forming elements as chromium is present near the leaner end of the range of 0.75% to 1.35%, carbon may likewise be present in an amount near 3.00%.

The excess carbon, over and above that which forms as carbide, and silicon are the primary elements which promote the depth of the chill. Very high carbon and high silicon increase the amount of graphite formed thereby leading to a decrease in the depth of chill. Further, silicon in excessive amounts results in the undesirable formation of soft pearlite in the micro-structure.

As indicated previously, optimum properties and performance are achieved through a proper balance of the chemistry. In the manner of carbon and silicon, and each further elemental addition acts individually or synergistically with another to enhance the properties or performance of the roll in a hot rolling application. For example, nickel in the iron helps to suppress pearlite formation while promoting the development of martensite. The high surface hardness of the rolls of this invention is gained through the additions of chromium and molybdenum. Chromium forms a stable carbide thereby assuring a proper balance between the nodular graphite and carbides in the chill portion of the roll. Molybdenum, on the other hand, increases the resistance of the roll's surface to spalling. Finally, magnesium is added to the chemistry of the chill portion to promote the formation of nodular graphite.

All of the preceding discussion has been directed to the chill portion of the composite cast iron roll. However, the greater bulk of the roll is the core portion. Early in the development of composite martensitic nodular graphite cast iron rolls there was considerable concern over the "marriage" between the chill portion and core portion. The outgrowth of this concern resulted in the preferred selection of a low alloy cast iron. By way of example, a preferred chemistry for the core was established, such chemistry consists essentially of, by weight.

|            |                |    |
|------------|----------------|----|
| Carbon     | 3.30% to 3.60% | 65 |
| Manganese  | 0.40% to 0.70% |    |
| Phosphorus | 0.10% max.     |    |
| Sulfur     | 0.05% max.     |    |
| Silicon    | 1.15% to 1.45% |    |
| Nickel     | 0.60% to 1.40% |    |

-continued

|          |                |
|----------|----------------|
| Chromium | 0.15% to 0.65% |
| Iron     | balance.       |

It has now been discovered that a suitable marriage can be made between the chill portion and a core portion whose chemistry varies from that given above. That is, variations to the core chemistry may be made so long as the core can withstand the rigors of a hot rolling application. As the core of a roll it must possess sufficient strength, ductility and toughness, the levels of which are well known. Additionally, the core must be machinable to provide proper journaling of the roll, while being wear resistant. A final factor in determining whether a suitable marriage can be effected between the chill portion and the core portion is the pouring practice. Two well known methods of manufacturing composite rolls are the centrifugally cast roll and the static sequential double poured rolls. Within each method the individual capabilities or pouring practices of a given roll foundry can effect the soundness of the roll, hence the marriage between the chill portion and the core portion. Thus, while the above tabular listing for the core chemistry is preferred, it should not be read as a limitation on this invention.

Following the selection of a balanced chemistry for the chill-cast surface portion and a core chemistry metallurgically compatible therewith, a roll may be cast in a manner known in the art. After solidification and cooling, the as-cast roll is subjected to a stress-relief treatment in the manner taught in U.S. Pat. No. 3,623,850. The roll may then be machined and dressed for use in hot rolling applications.

In order to establish the effectiveness of the roll of this invention under the severe temperature conditions of a hot strip mill, a lengthy trial was conducted on a hot strip mill. The trial covered seventeen weeks using rolls of the type described herein and rolls of the high-chromium variety. The purpose of the trial was to determine the maximum tonnage that could be rolled consistent with good surface quality with each roll. Typical analyses and hardnesses of the rolls in this trial are listed in Table I.

TABLE I

|              | Type Roll        |               |
|--------------|------------------|---------------|
|              | A*-High-Chromium | B**-Invention |
| Total Carbon | 2.52             | 3.35          |
| Mn           | .72              | .57           |
| P            | .046             | .050          |
| S            | .044             | .006          |
| Si           | .50              | 1.52          |
| Ni           | .39              | 4.05          |
| Cr           | 15.51            | .99           |
| Mo           | 2.41             | .65           |
| Mg           | —                | .05           |
| Hardness     |                  |               |
| Shore "C"    | 74               | 79            |

\*Commercially produced centrifugally cast roll - clear-chill iron roll with graphite-free white iron structure containing chromium carbides.

\*\*Static sequential double poured roll - indefinite-chill iron roll containing nodular graphite in a predominantly martensitic structure.

This rolling trial was limited to tinplate because this presents one of the most demanding roll applications and also to eliminate variables arising from product mix. Maximum strip width rolled was 40 inches (0.074 inch and 0.080 inch gauge). Roll lubrication was not used during the trial. Past experience on this mill had found that the maximum rollings of tinplate, using steel

cast rolls, were limited to about 750-1000 tons/run. Finally, on this hot strip mill which contains seven finish rolling stands in tandem, typical temperatures for the processing of tinplate in the finish rolling stands varies between 1900° and 1600° F. In the first three of such stands the work rolls typically are subjected to strip temperatures above about 1800° F.

In evaluating the performance of the rolls during and at the conclusion of the rolling, the rolls of this invention (B) and the high-chromium rolls (A) were nearly equivalent in tons rolled/0.001 inch dressing. In the second finishing stand, where the predominant mechanism of wear is by thermal fatigue, the roll of this invention was superior. That is, Roll B was found to be much less sensitive to thermal conditions in the mill. Where abrasive wear predominates, the high-chromium rolls (A) fared better. However, it is misleading to compare hot strip mill roll performance based strictly on wear rates. Since strip quality must be considered, the surface breakdown by roughening or banding is often the limiting factor. For example, in the fifth stand the high-chromium rolls (A) became very rough after rolling about 1300 tons (approximately 155,000 lineal feet). In contrast to this, the rolls of this invention (B) produced as much as 2100 tons (263,430 lineal feet) of tinplate exhibiting fairly even, light wear with minimal light banding.

It was discovered during the evaluation of a later trial that the results of the 17 week trial were not representative of the differences in performance of the two types of rolls on a commercial hot mill. The results were not representative in that the mill experienced only one cobble during the entire trial. As the product mix on a mill begins to vary in composition, more particularly in gauge and width, the frequency of cobbles goes up. The high-chromium rolls (A) are quite

5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

about 3.00 to 3.70% carbon, about 0.35 to 1.25% manganese, about 1.0 to 2.0 silicon, about 3.75 to 5.75% nickel, about 0.75 to 1.35% chromium, about 0.40 to 1.10% molybdenum, about 0.03 to 0.08% magnesium, the balance iron and incidental impurities, and

2. a core portion comprising a ferrous alloy whose chemistry and mechanical properties are metallurgically compatible with the chemistry and properties of said surface portion.

2. The process according to claim 1 wherein the hot rolling is effected at temperatures above about 1600°F.

3. The process according to claim 1 wherein the carbon is about 3.10 to 3.40%, manganese about 0.45 to 0.75%, silicon about 1.35 to 1.65%, nickel about 3.90 to 4.30%, chromium about 0.90 to 1.30%, and the molybdenum about 0.55 to 0.80%.

4. The process according to claim 1 wherein the surface portion has a hardness of at least 80 Shore-C.

5. The process according to claim 2 wherein the hot rolling is effected at temperatures above about 1800°F.

\* \* \* \* \*

15

20

25

30

35

40

45

50

55

60

65